

## UNITED STATES PATENT OFFICE

2,106,221

## PROCESS FOR THE REFINEMENT OF MAGNESIUM AND MAGNESIUM ALLOYS

Alexander Luschenowsky, Berlin, Germany

No Drawing. Application January 21, 1937,  
Serial No. 121,618. In Germany February 3,  
1936

3 Claims. (Cl. 75—67)

I have filed applications in Germany on the 3rd February, 1936 and 13th May, 1936; Austria on the 21st February, 1936; Hungary on the 28th February, 1936; Czechoslovakia on the 15th February 5 1936 and Switzerland on the 6th June 1936.

The present invention relates to processes for the refinement of magnesium and magnesium alloys.

In the U. S. A. Patent 2,067,275 a process for 10 the refinement of magnesium and magnesium alloys by means of hydrogen peroxide and also by means of hydrogen peroxide and hydrogen is described. According to the said process the magnesium or a magnesium alloy is treated by 15 passing through the molten metal vapours which are emitted by an aqueous solution of hydrogen peroxide, hydrogen being, if desired, led through the solution of hydrogen peroxide and then passed through the molten metal.

Now, I have discovered as a result of further 20 investigations that the efficiency of this process can be increased to a surprising extent if an oxide of manganese, such as manganese oxide ( $Mn_2O_3$ ) or manganese dioxide ( $MnO_2$ ), is added 25 to the aqueous solution of hydrogen peroxide, and according to the present invention the molten magnesium is treated with vapours which are emitted by an aqueous hydrogen peroxide solution to which an oxide of manganese as afore- 30 said has been added. Furthermore, the process according to the invention may be carried out in such manner that hydrogen is led through the aqueous solution of hydrogen peroxide to which an oxide of manganese has been added, and is 35 then passed into the molten metal.

The addition of manganese oxide ( $Mn_2O_3$ ) or manganese dioxide ( $MnO_2$ ) respectively to the solution of hydrogen peroxide causes more energetic 40 development of gas and assists the refinement or purification of the metal. It has been found that the process described enables reliable refinement of magnesium and magnesium alloys to be effected in a surprisingly short time, the melt being practically entirely freed from all the 45 substances to be removed (chlorine and in particular nitrogen compounds of magnesium). The magnesium refined according to the novel process exhibits a higher capacity for resisting corrosion as also better mechanical properties, and, 50 in particular, a considerably lower combustibility.

The process according to the invention is preferably carried out in the following manner:

The magnesium is melted up with a suitable 55 fluxing means. To a solution of hydrogen peroxide in water (for example a 2-15% solution) manganese oxide or manganese dioxide respectively (i. e.  $Mn_2O_3$  or  $MnO_2$  respectively) is added in powder form and well mixed in with the solution. The quantity of manganese oxide or man-

ganese dioxide respectively preferably amounts to 1-5% of the total weight of the liquid. This mixture is heated in a closed vessel to a temperature below its boiling point. By the aid of a conduit the vapours arising from the solution (hydrogen peroxide or its decomposition products respectively and water vapour) are passed into the molten magnesium or magnesium alloy. During this operation the supply conduit is gradually immersed more and more deeply in the melt and is caused to agitate the latter.

In similar manner the refinement may be carried out by leading hydrogen through an aqueous solution of hydrogen peroxide (for example a 1-12% solution), to which manganese oxide or manganese dioxide respectively ( $Mn_2O_3$  or  $MnO_2$  respectively) has been added in powder form in a quantity amounting to 1-5% of the total weight of the liquid, the latter being contained in a closed vessel, and is then passed into the molten magnesium or magnesium alloy as the case may be. During this operation, as previously described, the supply conduit which is provided at its lower end with perforations is gradually immersed more and more deeply in the molten metal and is employed at the same time for agitating the melt.

The refinement takes place very rapidly. With a crucible of 5 kg. capacity it only requires about 1 minute. The surface of the refined melt is as bright as a mirror. After the refinement the melt is allowed to stand for a few minutes after which the metal can be cast or poured without protection against gas or other protecting shields.

I claim:

1. A process for the refinement of magnesium and magnesium alloys, comprising in steps: melting the metal which is to be refined; and passing through the molten metal the vapours emitted by an aqueous solution of hydrogen peroxide containing an oxide of manganese.

2. A process for the refinement of magnesium and magnesium alloys, comprising in steps: melting the metal which is to be refined; and passing through the molten metal the vapours emanating from an aqueous solution of hydrogen peroxide which has been heated to a temperature below its boiling point and to which an oxide of manganese has been added in a quantity amounting to 1 to 5% of the total weight of the liquid.

3. A process for the refinement of magnesium and magnesium alloys, comprising in steps: melting the metal which is to be refined; and leading into the molten metal hydrogen which has been passed through an aqueous solution of hydrogen peroxide to which an oxide of manganese has been added in a quantity amounting to 1 to 5% of the total weight of the liquid.

ALEXANDER LUSCHENOWSKY.